

May 23, 1933.

S. O. COWPER-COLES

**1,910,150**

## APPARATUS FOR ELECTRODEPOSITION OF METALS

Filed May 6, 1930

2 Sheets-Sheet 1



Inventor:  
Casper Gles,  
By  
Davis & Davis, Elmont;  
His Attorneys.

May 23, 1933.

S. O. COWPER-COLES

1,910,150

APPARATUS FOR ELECTRODEPOSITION OF METALS

Filed May 6, 1930

2 Sheets-Sheet 2



 Inventor  
S. O. Cowper-Coles  
By  
Purcell, Dennis, Knobbe, E. G.  
His Attorneys

## UNITED STATES PATENT OFFICE

SHERARD OSBORN COWPER-COLES, OF SUNBURY-ON-THAMES, ENGLAND, ASSIGNOR TO  
F. C. METAL PROCESSES LIMITED, OF LONDON, ENGLAND, A BRITISH COMPANY

## APPARATUS FOR ELECTRODEPOSITION OF METALS

Application filed May 6, 1930, Serial No. 450,180, and in Great Britain May 15, 1929.

My invention has for its object the rapid and economical electro-deposition of metals, especially copper, of a quality superior to any hitherto attainable and in what I believe to be a new physical condition such that the deposited metal is at once and without further treatment suitable for the manufacture of a variety of industrial products as hereinafter indicated. The metal is of exceptional purity, density and hardness; thus, in the case of copper, a hardness numeral of 130 or more on the Brinell scale and a breaking stress in tension of 35 tons per square inch are obtainable. The process results in uniformity of structure owing to the fact that the metallic crystals are, to a large extent at least, broken down; any remaining crystals all lie in one direction, thus also conduced to uniformity. The metal may be obtained as sheet, strip or wire or in the form of cylinders or tubes of any desired diameter.

According to the invention the cathode employed for the electro-deposition of the desired metal is constituted by a horizontal mandrel rotated at a speed resulting in turbulence of the electrolyte sufficient to break up the film of exhausted electrolyte in proximity to the mandrel, rollers or discs free to revolve and capable of a limited movement in the circumferential direction of the mandrel being arranged to bear on the metal deposited thereon. The rollers are mounted on a carriage or the like which is moved to and fro in a direction parallel to the axis of the mandrel, the arrangement preferably being such that the rollers are operative during motion in one direction only. The above-mentioned qualities of the metal deposited may be varied by altering the pressure exerted by the rollers or discs or the number of to-and-fro movements performed in unit time, or by changing both these factors.

It will be realized that this invention differs essentially from that disclosed in my prior English specification No. 21,974 of 1898, in that in the latter case there is employed a vertical mandrel wholly immersed and rotated at a speed sufficiently high to throw off by centrifugal force the cathodic

film of exhausted electrolyte containing hydrogen bubbles, whereas in the present case the mandrel is only partially immersed and the speed is merely sufficient to lift, at the point at which the rotating surface of the mandrel emerges from the electrolyte, a small quantity of the electrolyte a few inches above the normal surface of the liquid, from which height it falls back giving the appearance of a cascade, producing agitation of the liquid and breaking up the cathodic film. The fact of the rollers being operative during axial travel in one direction only results in equality of treatment over the whole surface of the mandrel and causes the metal to be deposited in such a manner that any crystals which in the process are not broken down lie substantially in one direction, producing uniformity in the metallic structure hitherto, I believe, unattained. The rollers are preferably so mounted as to bear on the mandrel solely by their own weight, such pressure determining to a large extent the density and other qualities of the deposited metal; in order to vary the pressure rollers of different weights are preferably employed, but obviously such variation may be secured by means of spring pressure or weights applied to the frame or the like carrying the rollers.

In describing my invention I will take copper as the metal to be deposited from a suitable electrolyte such as sulphate of copper and in the first place I will describe the process as adapted for the manufacture of copper sheet. In a suitable vessel containing the electrolyte I mount the rotatable mandrel, so that about half of the circumference of the mandrel is below the surface of the electrolyte. Below the mandrel I place the anode which may consist of copper bars placed side by side so as to form a continuous semi-cylindrical conductor adjacent to and following the contour of the cylindrical surface of the mandrel, the space between the cathode and anode being about one quarter of an inch. The mandrel consists of a cylinder or drum which may be wholly or partly made of metal, but which has a polished metal surface that has been

treated in any known manner to prevent the adhesion of the deposited metal. A special method of treating the surface to prevent adhesion forms a subsidiary feature of my present invention. Suitable arrangements are made for rapidly rotating the mandrel at the critical speed above referred to, which, however, is not so high that any substantial part of the liquid is carried up and over the drum, but sufficient to cause the turbulence in the electrolyte necessary to break up the cathodic film as above described.

Bearing upon that portion of the mandrel which is not immersed in the electrolyte there are arranged revoluble rollers or discs of metal or glass or any other suitable material. In copper deposition I have found a very suitable material is a high-percentage ferro-silicon alloy which is not attacked by copper sulphate solution. The rollers or discs are so arranged that they exert a comparatively heavy pressure per unit area of contact on the deposited metal owing to the fact that that area is very small. In practice I have found it desirable to deposit a thin layer of copper before allowing the rollers or discs to be applied. The rollers or discs are free to rotate by frictional contact with the surface of the mandrel, (it being understood that in this term I include the metal deposited thereon,) and are also capable of a limited movement in the circumferential direction of the mandrel: I refer to them accordingly as "floating" rollers. Further, they are arranged and mounted so that they can be moved in contact with the mandrel transversely in a direction parallel its axis. The transverse movement of the rollers or discs is a reciprocating movement, but they should only contact with the mandrel when moved in one direction; the return movement should be out of contact therewith. The function of these rollers or discs is (1) still further to ensure the film of electrolyte on the mandrel being broken up and (2) at the same time through their rolling pressure and rubbing action, due to the transverse motion, to produce a deposit of copper which possesses an extraordinary degree of toughness. The consolidating effect of the rollers or discs also assists in eliminating any nodules or roughness which the deposited copper may tend to form, with the result that the latter presents throughout an unusually smooth and even surface.

One or more rows of rollers or discs may be fitted to bear upon the mandrel and in the case of long thin mandrels which have a tendency to sag I may find it expedient to arrange a row of rollers or discs underneath the mandrel and two rows on the top.

In order to prevent the deposition of metallic excrescences at the edges of the mandrel which renders the stripping of the sheets or tubes difficult, rapidly destroys the insulating

material, affects the speed of rotation and generally reduces the efficiency of the process, I place secondary electrodes at both ends of the mandrel. These secondary electrodes are semi-circular plates made of lead or other inert electrical conductors, or of wood, vulcanite or other insulating material or a combination of an insulating and conducting material capable of withstanding the electrolyte, so arranged that they are in close proximity to the mandrel and preferably provided with a flange to overlap a portion of its depositing surface. The effect of these secondary electrodes is that they reduce the rate of deposit at the extreme ends of the mandrel and instead of the metal building up at the ends, the deposit can be so regulated that the ends are just as smooth and the thickness of the deposited metal the same as on the other parts of the mandrel, or it can be arranged so that the deposit slightly tapers off. Again by making the secondary electrodes of the same metal as deposited on the mandrel the deposit may be thickened up at the edges.

In order to facilitate the detachment of the deposited metal from the mandrel, I form upon the metallic surface of the latter a film of oxide or sulphide; or a thin film of lead may be deposited thereon which may be highly polished with plumbago or other suitable polishing agent.

To avoid small holes or other imperfections in the deposited metal, which may be due to a medium applied to facilitate stripping or to other causes, I may find it desirable, after deposition for a comparatively short time and, before application of the floating rollers or discs, to cause a rapidly revolving brush to travel over the surface of the mandrel, whereby the thin deposit is levelled up and further deposit is free from flaws and blemishes. Preferably the mandrel is provided with a transverse groove or an insertion of a material of higher specific resistance than that on the mandrel surface as a whole, with the result that the deposit is locally thinner or even entirely absent, thereby furnishing a line along which stripping of the deposited sheet from the mandrel may be started.

Metal sheet produced in this way is so homogeneous and smooth that it is capable of being advantageously used for printing plates or gramophone discs or other purposes for which electro-deposited copper is not normally adapted.

The process of electro-deposition I have described is applicable to the production of tubes or cylinders. In the deposition of metal in the form of seamless tubes greater difficulty is sometimes experienced in detaching the tube from the mandrel than in the case where the removal of the deposited metal is effected by stripping it off from the mandrel as a sheet or strip. I have found that in order to ensure the ready detachment of a

tubular deposit it is advantageous to use copper or brass-coated mandrels which have their surfaces highly polished and are then coated with a solution containing 0.05% to 5 0.5% of beeswax dissolved in turpentine, to which solution 1% of carbon bisulphide is added. The same composition may be used, if desired, to facilitate the detachment of sheets or strips.

10 In order to obtain a surface on the mandrel which at reasonable cost will ensure that the inner surface of the deposited sheet, (that is the surface in contact with the mandrel), is perfectly smooth and free from imperfections, I construct the mandrel or drum of 15 welded steel or iron sheet or cast iron, which is then turned and polished. On this surface I then electro-deposit copper, having first made the surface passive by treatment with 20 nitric acid or other well-known means so as to ensure the adherence of the copper deposited. Upon a mandrel having a surface so prepared, polished and treated with a preparation for facilitating detachment I am 25 then able to deposit copper according to the process herein described to produce sheets, tubes or cylinders whose inner surface is mirror-like and whose outer surface also is unusually smooth and free from imperfections. 30 I produce copper strip or wire having the special characteristics obtainable in accordance with the present invention in the following way. I form upon the surface of the mandrel a helically disposed V-shaped groove 35 as described in my prior specification No. 21,568 of 1904,—the pitch of the helix corresponding with the width of the strip which it is desired to produce. The V-shaped groove forms a weak line of cleavage in the 40 deposited metal, enabling it to be removed from the mandrel in the form of a continuous strip, which may then be rolled or drawn through draw plates or dies to form wire.

The copper strip as unwound from the 45 mandrel has a small fin on either edge due to fission along the line of cleavage in the metal deposited in the V-shaped groove. Unless special means are taken to eliminate this fin it is apt to result in imperfect wire. I find 50 that the best means to eliminate it is to run the strip in the process of stripping off from the mandrel between rollers which are so shaped or are set at such an angle that they press the small fins into the body of the strip 55 so that when it is drawn through a round die there is no fear of the fins turning over and forming lines or imperfections in the finished wire.

For the purpose of my invention I use any 60 of the electrolytes ordinarily used for the deposition of the metals to which my invention relates. I find, however, that in depositing copper according to my invention an advantageous electrolyte for certain purposes 65 consists of a strong, almost saturated, solu-

tion of the sulphate of aluminium, magnesium or other alkaline metal, to each gallon of which is added about 5 ozs. of copper sulphate and a volume of sulphuric acid of about the same weight. I find that this electrolyte 70 gives remarkably smooth, homogeneous and ductile deposits and it can be worked at a high current density and low voltage; for instance at 100 amperes or more per square foot, the voltage at the terminals of the cell 75 being in the order of 0.8. The solution is preferably worked hot at a temperature of about 90° C. If a copper anode is used in such a solution it dissolves away evenly leaving a smooth surface. 80

It will be realized that in the case of all the above described operations the anode constitutes the source of the metal which is deposited on the revolving cathode, the electrolyte merely acting as a vehicle for the transfer of this metal. It is, however, possible to employ the electrolyte as the source of the deposited metal, the anode, if desired, being made of lead, carbon, ferro-silicon or other electro-chemically inert material. The possibility is thus afforded of obtaining by an electrolytic method a metal directly from a compound containing it provided that such compound can be obtained in the form of a solution or held in suspension in a liquid 90 which is suitable to constitute an electrolyte. Thus a metal may be recovered directly from its ore without the necessity of a smelting process; for example, in order to recover copper from a sulphide ore in this manner I may proceed as follows:— 100

The ore is first concentrated by any of the well-known methods and if such method has necessitated the use of oil this must be removed by treatment with a suitable solvent or by applying the necessary heat. The concentrated ore is then mixed with a sodium chloride solution of a strength of about 10% and the sludge and the ore from the solution are circulated through a tank in which, as above described, is a horizontal revolving cathode and an anode composed of graphite or other suitable material. The solution with the ore in suspension is caused to circulate in the intervening annular space so that the copper sulphide is attacked by the nascent chlorine and converted into a cuprous copper chloride—the copper being deposited on the revolving cathode. In this way it is found possible to work at a very high current density—say, 200 amps. per square foot—with a low voltage and, on account of the solution being maintained in a cuprous state by any of the well-known methods, to obtain practically double the weight of deposited copper for a given current density that is possible in the case of a cupric solution; the voltage is also low—considerably under one volt. In place of the sodium chloride a sulphuric acid solution may be used, the sulphide metal be- 110 115 120 125 130

ing reduced with evolution of sulphuretted hydrogen and the sulphur finally recovered.

In the case of an ore containing different

metals, it may be possible, by what might be termed fractional electrolyzation, that is to say, by altering the conditions under which the electrolytic process is carried out, successively to obtain a deposit of each of the metals in a pure state. For example, in treat-

10 ing a sulphide ore containing nickel 4%, copper 9% and cobalt 2% the ore or concentrate is first roasted in a suitable furnace to a bright red heat with constant stirring until the sulphate state is reached. The roasted ore is

15 leached first with water and then with 10% sulphuric acid solution, the temperature not being allowed to rise above 30° C. After the desired extraction has been obtained, the solution is decanted and contains the copper

20 and cobalt, the nickel remaining in the residue. The latter is subjected to a further leaching operation with 10% sulphuric acid at 90° C. to extract the nickel and the solution is then electrolyzed in the manner above de-

25 scribed at a temperature of 80° C.; an insoluble anode is used and a voltage applied sufficient to result in a current density of about 60 amps. per square foot, whereupon the nickel is deposited as a cylinder which

30 may be stripped off in the form of sheet.

The first leaching solution containing the copper and cobalt salts is electrolyzed at a temperature of 30° C. and current density about 10 amps. per square foot with acidity 35 6% free acid and, using an insoluble anode, the cobalt is deposited on a suitable revolving cathode. When all the cobalt has been removed another revolving cathode is substituted, the current density is raised to 30 amps. 40 per square foot, the temperature to 60° C. and the acidity to about 9-10% free acid, when copper is obtained by deposition on the cathode, the iron in solution being crystallized out from time to time.

45 In all cases I have found it possible to operate economically at a higher current density than has hitherto been commercially employable; such current density is obtainable by the application of voltages substantially 50 lower than those used heretofore, due largely to the efficient depolarization and continual renewal of the cathodic film secured by running the rotating cathode at the critical speed above mentioned.

55 The mechanical features of the apparatus required for carrying out my invention may take various forms. A form of apparatus which I have found suitable is one in which the mandrel is supported by means of trunnions mounted in bearings outside the depositing tank. As current, which is of considerable magnitude, passes from the mandrel or drum through these bearings I provide for their being water-cooled and lubricated by means of graphite or other electrical

ly conductive lubricant. Alternatively, the current may be led to and from the mandrel by means of brushes and slip-rings.

I find a convenient means for the movement of the rollers or disc is the use of reversing-screw mechanism of well-known character, but, as hereinafter mentioned, other devices may be employed.

70 In order that the invention may be clearly understood and readily carried into effect it 75 will now be described more fully with reference to the accompanying drawings which illustrate various forms of apparatus for depositing metal having the unique qualities attainable in accordance with the invention, 80 and wherein:—

Figures 1 to 3 show respectively in side view, end view and plan apparatus suitable for depositing metal on a mandrel of comparatively large diameter with a view to its 85 subsequently being stripped off in the form of a sheet.

Figures 4 and 5 respectively illustrate in section two forms of floating rollers or discs for bearing on the mandrel.

90 Figures 6 and 7 depict an alternative mechanism for producing the to-and-fro transverse movement of the rollers or discs,

Figures 8 and 9 show in section and dia- 95 grammatic plan respectively apparatus suitable for the manufacture of tubes,

Figures 10 and 11 depict respectively in side view and end view rollers whereby the fin existing on a strip which has been deposited on the helically grooved mandrel and subsequently stripped off may be disposed of, Figures 12 and 13 being respectively sections of the said strip before and after treatment by the rollers.

100 Referring to Figures 1 to 3, the mandrel 1 is mounted within a suitable vat or the like 2, which is preferably lead lined, by means of a shaft 3 supported in bearings 4 vertically adjustable by means of screws 5 passing through suitably threaded supports 6. As indicated, the bearings 4 are preferably open-topped to facilitate ready removal and replacement of the mandrel 1 and, on account

105 of the fact that current is fed to the mandrel through the bearings, they are lubricated with graphite, or other electrically conductive lubricant, being preferably, also in view of the large current to be transmitted, water-cooled by means of ducts 7 connected by pipes 8 with a water supply. To relieve pressure on the bearings, the mandrel may be made hollow and watertight, so that a portion of its weight is taken by flotation in the electrolyte, the level of which is conveniently about as indicated in Figure 2. The mandrel is rotated by means

110 of a pulley 9, or analogous driving member, from a counter-shaft 10, which also, by means of worm gearing 11, serves to rotate a cam shaft 12 the purpose of which will be hereinafter described. The anode 13 constituted

115

120

125

130

by a copper casting or sheet or, as indicated in Figure 2, by a series of copper bars is in the form of an arc of a cylinder surrounding the lower portion of the mandrel which constitutes the cathode, being supported in this position by means of cradles or like members 14 which rest on the edge of the vat 2. In proximity to the ends of the mandrel there are arranged secondary electrodes 15 preferably, as indicated in Figure 2, of approximately semi-circular form and provided, as shown, with inwardly directed flanges of lead or other inert material which protrude between the edge of the mandrel and the anode 13. The secondary electrodes 15 are supported by means of rods or like members 16 which are attached to the bearings 4 by means of adjusting nuts 17; thus the distance of each secondary electrode from the end of the mandrel may be varied in order to produce the different effects as regards the thickness of the deposit above mentioned. It will be seen that, as the secondary electrodes are supported from the bearings 4, they partake in any vertical adjustment of the position of the mandrel 1 relatively to the anode 13 which may be given effect to in order to obtain the desired current density or to compensate for wastage of the anode 13.

The floating rollers or discs 18 bearing on the mandrel are carried on a spindle 19 supported by two bars 20 adapted to rock on a pivot bar 21 but prevented from moving endwise thereon by collars 22 fixed on the bar. A wiper 23 is also preferably loosely pivoted to the spindle 19 in such a position as to make contact with the mandrel just before it passes under the rollers 18 for the purpose of removing any grit, dirt or other extraneous matter which might have found its way into the electrolyte. The pivot bar 21 is journalled in bearings 24 supported in uprights 25 so that it is free to move in an axial direction for the purpose of producing the desired transverse travel of the rollers or discs 18 across the mandrel 1. To effect this movement the cam shaft 12 is provided with a snail cam 26 adapted to co-operate with a roller 27 provided on a lever 28 pivoted at 29 and connected by a link 30 with the pivot bar 21; thus rotation of the cam 26 results in travel of the rollers or discs 18 at a uniform rate across the mandrel 1 in a direction from left to right as seen in Figure 1, and upon reaching the right-hand end of the mandrel the lever 28 together with its associated members, is allowed to be drawn back rapidly toward the left by the action of a weight 31 connected with the pivot bar 21 by a cord or the like 32 passing over a pulley 33 as indicated: excessive shock due to rapid motion of the lever, pivot bar and rollers may be prevented by the provision of a suitable spring buffer 34. In order that, on the return stroke, the rollers or discs 18 shall be out of contact with the mandrel 1, they are lifted by means of a second cam 35 operating through a lever 36 pivoted at 37 and connected by a link 38, having a double knuckle joint 39, with a tipping bar 40 supported in arms 41 hinged around the pivot bar 21, the said tipping bar 40 bearing on the upper side of the rear end of the bars 20. The cam 35 is, as indicated, so shaped that during a short period of its revolution the lever 36 is depressed with the result that the rollers or discs 18 are raised from contact with the mandrel this action being timed to take place synchronously with the return transverse movement of the rollers or discs. As indicated, the vat 2 is preferably supported by insulators 42 and suitable means, not shown, are provided for making electrical supply connections respectively with the bearings 4 and the anode 13.

In order that the rollers or discs 18 may individually have freedom not only to revolve but of movement in the circumferential direction of the mandrel, the constructions shown by way of example in Figure 4 or Figure 5 may be adopted. Referring to Figure 4, each roller 18 is formed with a central aperture 43 of a diameter larger than that of the spindle 19, the rollers being preferably separated by distance-pieces 44. According to the construction depicted in Figure 5, the spindle 19 is surrounded by a bush 45 free to revolve thereon and the spaces enclosed within the apertures 43 in the discs 18 and the bush are filled with sponge rubber 46 whereby the desired freedom of movement of the individual rollers is permitted.

In the alternative form of transverse travel mechanism shown in Figures 6 and 7, the pivot bar 21 is stationary and the bars 20 are capable of sliding movement along it. Parallel to and on each side of the pivot bar 21 are screwed spindles 47 and 48 which are either rotated in opposite directions, as described below, or formed with oppositely handed threads. The bars 20 are provided with half-nuts 49 and 50 adapted respectively to co-operate alternatively with the spindles 47 and 48, the engagement of one half-nut or the other with its co-operating spindle being determined by the lie of a pivoted weight 51 adapted to oscillate between pins 52 fitted between the bars 20. The spindle 47 is the one whereby the operative transverse movement of the rollers 18 is produced, the spindle 48 being employed to effect the return stroke: consequently, it is desirable that the latter spindle shall revolve more rapidly than the former. The spindle 48 may be driven from the counter-shaft 10 or from any other suitably placed shaft by means of a cord or chain 53 passing over a pulley 54 on the spindle 48. A second pulley 55 on this spindle serves to drive, by means of a cross cord or belt 56, a pulley 57 of larger diameter

fitted on the spindle 47. In order to effect reversal at the ends of the forward and return strokes stationary cam plates 58 are provided to engage the pivoted arm on which the weight 51 is mounted, thereby throwing over this weight from contact with one of the pins 52 to contact with the other pin and so rocking the bars 20 to disengage the half-nut in operative relation with one of the 5 screwed spindles and engage the other half-nut with its spindle. The bars 20 are preferably provided with a counterweight 59 so that the pressure of the rollers or discs 18 on the mandrel 1 is determined wholly or to 10 any desired extent by the weight of the rollers themselves.

In the apparatus shown in Figures 8 and 9, two mandrels are employed each having a corresponding set of floating rollers 18 carried by a common frame 60 resting on a pivot bar 21 and adapted to be tilted on the return stroke by means of a tipping bar 40 as in the modification above described. As, 15 however, in the manufacture of tubes the length of the mandrels 1 may be very considerable, it is possible that sagging might be produced as a result of the pressure of the rollers 18. Consequently, a supplementary set of floating rollers 61 is provided on the 20 underside of the mandrels in order to afford them some degree of support. The set of rollers 61 is supported by means of a rod 62 adapted to slide vertically through the frame 60 and provided with a wing-nut or the like 25 whereby the upward pressure of a spring 64 serving to support the rod 62 and rollers 61 may be deposited. In order that, on the return stroke, the rollers 18 may be lifted from their respective mandrels by the tilting of the frame 60, it is obviously necessary that the rollers 61 shall be lowered out of contact with the mandrels 1 and this result is attained automatically by means of a collar 65 30 fitted on the rod 62 and provided with an inclined surface 66 adapted to co-operate with a similarly shaped surface on a sleeve 67 loose on the rod 62 and bearing against a fixed abutment 68 in such a manner that 35 rotation of the sleeve 67 results in depression of the rollers 61. The sleeve 67 is provided with an outwardly projecting rod 69 which, on the forward or operative stroke of the rollers 18 and 61, occupies the position relatively to the frame 60 shown in full lines in 40 Figure 9. On approaching the end of the operative stroke however, the rod 69 encounters a stop pin 70 and thereby, on account of the continued transverse travel of the frame 60, the rod 69 is retarded and 45 brought to the position shown in dotted lines so rotating the sleeve 67 and depressing the rollers 61. The tipping bar 40 then operates to tilt the frame 60 and the reversing mechanism comes into action to perform the return stroke, whereupon the rod 69 on ap-

proaching the end of that stroke encounters a second stop pin, not shown, which restores it to its original full-line position, thereby allowing the spring 64 to raise the rollers 61 into contact with the mandrels 1 at the same 50 moment as the tipping bar 40 is operated to allow the rollers 18 to bear on the mandrels.

The apparatus for removal of the fins which essentially exist on a strip or wire produced by depositing metal as above on a helically grooved mandrel and subsequently stripping it off, depicted in Figures 10 and 11, comprises essentially two rollers 71 and 72, the former of which is provided with a rectangular groove to accommodate that side 55 of the strip or wire on which the fins do not exist, that is to say, the lower portion of the wire a section of which before treatment is shown in Figure 12. The second roller 72 is formed with a groove, the bottom of which is bevelled, as indicated at 73 in Figure 11, so that wire of a section shown in Figure 12 when passed between the rollers has its section altered to that depicted in Figure 13. The outline of the original section is indicated in Figure 11 in dotted lines and it will be seen that between that portion of the upper surface of the wire intermediate of the fins and the opposing bottom of the groove in the roller 72 there is a space, this being provided to enable the fins to be squeezed by the bevelled portions 73 of the groove into the body of the wire rather than folded over on the outside thereof. The result is that the 60 above mentioned intermediate surface of the wire is forced outwards to fill the space above referred to as that the section of the wire, as illustrated in Figure 13, corresponds with the space between the rollers 72 and 73 constituted by the respective grooves in these 65 rollers. It will be realized that instead of employing a single roller 72, two rollers set at an angle and adapted to operate one on each fin may be employed, the peripheries of the rollers being shaped so that their combined action in co-operation with the roller 71 in disposing of the fins is similar to that 70 above described.

While the process and apparatus have been described more particularly in their application to the production of copper sheet, tubes, strip or wire, the invention is also applicable to the deposition of other metals such, for example as zinc, nickel, cobalt or silver, whether from their ores or other compounds as above indicated or by transfer from an anode of the metal in question.

What I claim and desire to secure by Letters Patent of the United States is:—

1. Apparatus for the electro-deposition of metal comprising a vat for containing the electrolyte, an anode immersed therein and a cathode in the form of a rotating mandrel on which rollers, free to revolve and capable of a limited movement in the circumferential 125

direction of the mandrel are adapted to bear, means being provided for moving the rollers to and fro transversely of the rotating mandrel, and for lifting the rollers out of contact with the mandrel during their transverse motion in one direction.

2. Apparatus as in claim 1, in which means is provided whereby the transverse movement of the rollers is comparatively slow in one direction followed by a rapid return movement.

3. Apparatus as in claim 1, wherein the transverse to and fro motion of the rollers is produced by cam-and-lever mechanism.

4. Apparatus as in claim 1, wherein the transverse to and fro motion of the rollers is produced by reversing screw mechanism.

5. Apparatus as in claim 1 in which cam-and-lever mechanism is provided for lifting the rollers out of contact with the mandrel during their transverse motion in one direction.

6. Apparatus as in claim 1, in which the rotating mandrel is provided with a shaft mounted in bearings located outside the vat and vertically adjustable by such means as a screw.

7. Apparatus as in claim 1, wherein the rollers are supported by a frame constituted by bars transverse to the axis of the mandrel and carried by a pivot bar about which it may rock and which permits of its transverse movement across the mandrel and the frame is extended on the side of the pivot bar remote from the rollers and is adapted to co-operate with a tipping bar whereby, on the return transverse stroke, the rollers are raised from contact with the rotating mandrel.

8. In apparatus as in claim 1, means for permitting the circumferential movement of the rollers according to which they are mounted on a common spindle which passes through an aperture in each roller substantially larger in diameter than that of the spindle.

9. In apparatus as in claim 1, means for permitting the circumferential movement of the rollers according to which they are mounted on a common spindle surrounded by a bush free to revolve, the spindle and bush passing through an aperture in each roller of substantially greater diameter than the external diameter of the bush and filled with resilient material such as sponge rubber.

10. Apparatus as in claim 1, in which a set of rollers is arranged to bear on the underside of the mandrel.

11. Apparatus for the electro-deposition of metal, comprising a vat for containing the electrolyte, an anode immersed therein, a cathode in the form of a rotating mandrel on the upper surface of which rollers, free to revolve and capable of a limited move-

ment in the circumferential direction of the mandrel, are adapted to bear, a set of rollers arranged to bear on the underside of the mandrel, means for automatically lowering the set of rollers bearing on the underside of the mandrel and subsequently raising the rollers bearing on the upper side of the mandrel, and a common frame capable of transverse motion for supporting the rollers bearing on the upper side of the rotating mandrel and those bearing on the underside thereof.

12. Apparatus as in claim 11, wherein a spindle supporting the rollers bearing on the underside of the mandrel is provided with a collar having a cam surface adapted to co-operate with a corresponding surface on a member which is automatically moved as each end of the transverse stroke is approached, whereby the spindle is depressed and the rollers lowered out of contact with the mandrel.

SHERARD OSBORN COWPER-COLES.

90

95

100

105

110

115

120

125

130